# EUROPEAN PATENT SPECIFICATION

(11) **EP 1 531 175 B1**
(45) Date of publication and mention of the grant of the patent: **30.03.2016**
(21) Application number: 04026422.8
(22) Date of filing: 08.11.2004
(51) Int. Cl.: C10M 129/16, C10M 145/36, C10M 141/02, C10M 141/06, C10M 161/00, C10M 163/00, C10M 165/00, C10N 40/04

(54) **Compositions and methods for improved friction durability in power transmission fluids**
Zusammensetzungen und Verfahren für die verbesserte Beständigkeit der Reibungseigenschaften von Getriebeölen
Compositions et méthodes permettant d'améliorer la durabilité du frottement dans des liquides de boîte de vitesses

(30) Priority: 12.11.2003 US 705992
(43) Date of publication of application: 18.05.2005
(73) Proprietor: Afton Chemical Corporation, Richmond, VA 23219 (US)
(72) Inventor: Saathoff, Lee D., Glen Allen Virginia 23060 (US); Tersigni, Samuel H., Glen Allen, VA 23060 (US); Yatsunami, Kenji, Tokyo, 107-0062 (JP)
(74) Representative: Dunleavy, Kevin James

(56) References cited:
- EP-A- 0 761 804
- FR-A- 1 445 009
- GB-A- 1 462 287
- GB-A- 2 285 056
- US-A- 3 679 588
- US-A- 4 968 453
- US-A1- 2002 002 118

## Description

### FIELD

The present invention relates to transmission fluid compositions and methods for incorporating an alkoxylated alcohol component in power transmission fluids that provide high overall friction and improved friction durability, yielding effective transmission fluids that are stable with age and operating stresses. The present invention also relates to methods for measuring friction performance of a power transmission fluid.

### BACKGROUND

Power transmission fluids must serve many functions, including the capability to provide sufficient coefficients of friction for friction plates, and in the case of a continuously variable transmission (CVT), the proper steel-on-steel coefficient of friction.

Considerable effort has been devoted to the provision of oil-soluble additive formulations for use in power transmission fluids, and in particular those for automatic transmissions and CVTs. Friction modifiers have frequently been used in such formulations to modify the shape of the "friction vs. sliding speed" curve (the µ-v curve), in general, to make it more positive. One disadvantage of many friction modifiers is that they typically deteriorate with thermal and chemical stresses. This can lead to shudder in slipping torque converters, in lock-up torque converters, in shifting clutches, in clutch-to-clutch transmissions, and in transmissions with wet starting clutches. It can also lead to instability in measures of dynamic friction in three-, four-, five-, six-, or seven-speed transmissions, and in CVTs (chain, belt, or toroidal disk type). There is a need for a highly stable friction modifier as an additive in a power transmission fluid that would extend its useful life.

EP-A 761 804 A1 discloses lubricating compositions which may include a base oil, at least one molybdenum compound, and a (poly)glycerol ether and/or a (poly)oxyalkylene glycol monoalkyl ether. These lubricating compositions may optionally further include a variety of other additives including dispersants and may be used as automobile transmission fluids.

U.S. Patent no. 3,679,588 discloses petroleum based hydraulic fluids containing a combination of additives including a Mannich dispersant and polyoxyethylene lauryl alcohol.

U.K. Patent application no. GB 2 285 056 A discloses a friction improving additive for an oil-based automatic transmission or wet brake fluid formed by heating at least one ashless dispersant which contains basic nitrogen and/or at least one hydroxyl group with a combination of (i) an inorganic acid of phosphorus, (ii) a boron compound, and (iii) a polyol having less than 12 carbon atoms to form a liquid composition. In examples, a commercial succinimide dispersant is reacted with phosphorous acid, boric acid and 1,2-propylene glycol.

### BRIEF DESCRIPTION OF EMBODIMENTS

The present invention discloses the novel use of an alkoxylated alcohol of the formula R-[O-(CH₂)_{X}]_{Y}-OH, wherein R is a C₈-C₁₈ aliphatic hydrocarbon group, X is 2 to 4, and Y is 1 to 6, in combination with a dispersant selected from a hydrocarbyl succinimide, a hydrocarbyl succinamide, a mixture of an ester and an amide of a hydrocarbyl-substituted succinic acid, and a hydroxyester of a hydrocarbyl-substituted succinic acid, as a friction modifier in a power transmission fluid that achieves improved friction durability relative to a fluid having the same composition absent said at least one alkoxylated alcohol. Further, the power transmission fluids of the present disclosure may provide improved or lower static friction while maintaining dynamic friction, thus controlling (or decreasing) friction in a stable manner.

In an embodiment, a power transmission fluid having improved friction properties, may comprise a major amount of a base oil and a minor amount of an additive composition including at least one alkoxylated alcohol of the formula R-[O-(CH₂)_{X}]_{Y}-OH, wherein R is a C₈-C₁₈ aliphatic hydrocarbon group, X is 2 to 4, and Y is 1 to 6, in combination with a dispersant selected from a hydrocarbyl succinimide, a hydrocarbyl succinamide, a mixture of an ester and an amide of a hydrocarbyl-substituted succinic acid, and a hydroxyester of a hydrocarbyl-substituted succinic acid, as a friction modifier in a power transmission fluid that achieves improved friction durability relative to a fluid having the same composition absent said at least one alkoxylated alcohol. The transmission fluid contains 0.01-20 wt.% of the alkoxylated alcohol and 0.01-15 wt.% of the dispersant, based on the total weight of the transmission fluid.

In another embodiment, a method of making a power transmission fluid concentrate having improved friction modifying properties may comprise combining at least one alkoxylated alcohol of the formula R-[O-(CH₂)_{X}]_{Y}-OH, wherein R is a C₈-C₁₈ aliphatic hydrocarbon group, X is 2 to 4, and Y is 1 to 6, and a dispersant selected from a hydrocarbyl succinimide, a hydrocarbyl succinamide, a mixture of an ester and an amide of a hydrocarbyl-substituted succinic acid, and a hydroxyester of a hydrocarbyl-substituted succinic acid and heating the alkoxylated alcohol and the dispersant at a temperature between 25 °C and 200 °C for a time between 0.1 to 196 hours.

In another embodiment, a method of making a power transmission fluid may comprise combining an alkoxylated alcohol of the formula R-[O-(CH₂)_{X}]_{Y}-OH, wherein R is a C₈-C₁₈ aliphatic hydrocarbon group, X is 2 to 4, and Y is 1 to 6, with a dispersant selected from a hydrocarbyl succinimide, a hydrocarbyl succinamide, a mixture of an ester and an amide of a hydrocarbyl-substituted succinic acid, and a hydroxyester of a hydrocarbyl-substituted succinic acid, and forming a mixture, heating the mixture, and adding the mixture to a base oil.

In another embodiment, a method of making a power transmission fluid may comprise combining an alkoxylated alcohol of the formula R-[O-(CH₂)_{X}]_{Y}-OH, wherein R is a C₈-C₁₈ aliphatic hydrocarbon group, X is 2 to 4, and Y is 1 to 6, with a dispersant selected from a hydrocarbyl succinimide, a hydrocarbyl succinamide, a mixture of an ester and an amide of a hydrocarbyl-substituted succinic acid, and a hydroxyester of a hydrocarbyl-substituted succinic acid, and forming a mixture, and adding the mixture to a base oil to provide a transmission fluid containing from 0.01-20 wt.% of the alkoxylated alcohol and 0.01-15 wt.% of the dispersant.

### BRIEF DESCRIPTION OF THE DRAWINGS

**FIG. 1(A)** illustrates friction profiles for samples tested in a LFW-1 test according to some embodiments of the present disclosure.
**FIG. 1(B)** illustrates friction profiles for samples tested in a LFW-1 test according to some embodiments of the present disclosure.
**FIG. 2** illustrates friction profiles for samples tested in a LFW-1 test according to some embodiments of the present disclosure.
**FIG. 3** illustrates friction profiles for samples tested in a LFW-1 test according to some embodiments of the present disclosure.

### DETAILED DESCRIPTION OF EMBODIMENTS

Novel compositions for enhancing friction and friction durability in power transmission fluids, and also methods for making and using these compositions are presented herein. The power transmission fluids of the present disclosure may comprise a major amount of base oil and a minor amount of an additive composition including an alkoxylated alcohol or mixture of alkoxylated alcohols of the formula R-[O-(CH₂)_{X}]_{Y}-OH, based on the total weight of the fluid, wherein R is an aliphatic hydrocarbon group having from 8 to 18 carbon atoms, X is 2 to 4, and Y is 1 to 6; and a dispersant selected from a hydrocarbyl succinimide, a hydrocarbyl succinamide, a mixture of an ester and an amide of a hydrocarbyl-substituted succinic acid, and a hydroxyester of a hydrocarbyl-substituted succinic acid. The present compositions achieve improved performance and friction durability in power transmission fluids through the incorporation of 0.01 to 20 wt.% of the alkoxylated alcohol component, which enhances the life of a transmission fluid that is subjected to oxidative and thermal degradation conditions during normal service.

The present embodiments overcome previous difficulties in achieving enhanced friction performance and overall utility of a power transmission fluid over long periods of time.

The alkoxylated alcohol friction modifiers useful in embodiments of the present disclosure are represented by the general formula:

R-[O-(CH₂)_{X}]_{Y}-OH

wherein R may be a linear, branched, or cyclic aliphatic hydrocarbon group having from 8 to 18 carbon atoms, X may range from 2 to 4, and Y may range from 1 to 6.

As used herein, a "power transmission fluid" or "transmission fluid" may include a lubricant useful for contact with gears involved in the transmission of mechanical energy, including in transmissions that may contain a slipping torque converter, a lock-up torque converter, a starting clutch, and/or one or more shifting clutches. Such transmissions may include a three-, four-, five-, six-, or seven-speed transmission, or a continuously variable transmission (chain, belt, or toroidal disk type) or a manual or an automatic transmission.

In an embodiment, the present invention achieves improved friction performance and durability of friction performance in power transmission fluids through the incorporation of 0.01 to 20 wt.% of the alkoxylated alcohol friction modifier component that is both effective and stable over a long period of time. It is contemplated that the alkoxylated alcohol component may comprise one species of a particular alkoxylated alcohol (e.g., ethoxylated lauryl alcohol, or "ELA"), or a mixture of alkoxylated alcohols within the scope of the present disclosure.

In an embodiment of the present invention, the alkoxylated alcohol component may be added to a power transmission fluid as one constituent in an overall formulation. In another embodiment, alkoxylated alcohol may be added to the power transmission fluid in conjunction with another transmission fluid additive, such as a dispersant. In an embodiment of the invention, the alkoxylated alcohol is added to the transmission fluid or to the additive package with no processing or reacting. In another embodiment, the alkoxylated alcohol is first heated with an ashless dispersant and the resulting mixture is then added to the transmission fluid or additive package.

In an embodiment, the additives provided by this disclosure provide for the incorporation of an alkoxylated alcohol component to a power transmission fluid at room temperature, and at no particular interval in the processing sequence. Once prepared, this novel additive imparts improved friction characteristics, and importantly, provides these benefits over the life of the fluid. Another embodiment provides for the combining and heating of the alkoxylated alcohol component with a dispersant prior to incorporation of the mixture in the power transmission fluid. The dispersant may contain either or both phosphorus and boron, or neither phosphorous nor boron.

As described herein, dispersants may comprise ashless dispersants that may be a hydrocarbyl-substituted succinimide, a hydrocarbyl-substituted succinic acid, a hydrocarbyl-substituted succinamide, a mixture of an ester and an amide of a hydrocarbyl-substituted succinic acid, and a hydroxyester of a hydrocarbyl-substituted succinic acid. Typical hydrocarbyl succinimides are disclosed in the following U.S. patents: U.S. 3,018,247; U.S. 4,554,086; and U.S. 4,857,214. Mixed ester-amides of hydrocarbyl-substituted succinic acids using alkanols, amines, and/or aminoalkanols are described, for example, in U.S. 4,234,435. The use and preparation of hydrocarbyl-substituted succinic acid esters and succinic acid salts are disclosed, for example, in U.S. 3,275,554; U.S. 3,454,555; and U.S. 3,565,804.

The dispersant used in an embodiment of the present disclosure may comprise hydrocarbyl succinimides in which the hydrocarbyl substituent is a hydrogenated or unhydrogenated polyolefin group; and in a particular embodiment, a polyisobutylene group having a number average molecular weight (measured by gel permeation chromatography) ranging from 700 to 10,000, and in another embodiment ranging from 700 to 5,000, and in another embodiment ranging from 750 to 2,500. The overall amount of dispersant used in an embodiment may range from 0.01 wt% to 15 wt%, or as another example, from 0.01 wt% to 10 wt%. In another embodiment, the amount of dispersant used in a power transmission fluid may range from 1 wt% to 8 wt%. Another embodiment may include the dispersant at ranges from 2 wt% to 6 wt%.

A process for preparing the transmission fluid additives may comprise combining in any sequence an alkoxylated alcohol or mixture of alkoxylated alcohols with a transmission fluid. Another embodiment may include a process that comprises combining in any sequence an alkoxylated alcohol or mixture of alkoxylated alcohols with a dispersant and heating at a temperature that ranges between 20°C and 200°C for a time ranging from 0.1 to 196 hours. As a further example, the combination may be heated at 60 °C to 170 °C. As an even further example, the combination may be heated for 0.5 to 24 hours. In an embodiment, the dispersant may be treated with a boron- and/or a phosphorus-containing compound either prior to, concurrently, or following the addition of the alkoxylated alcohol component.

The concentration of the alkoxylated alcohol component in the finished transmission fluid may range from 0.01 wt% to 20 wt%, as a further example, from 0.05 wt% to 10 wt%, as an even further example, from 0.1 wt% to 6 wt%, and as an even further example, from 0.1 wt% to 3 wt%. In an embodiment in which the ashless dispersant is combined with the alkoxylated alcohol prior to adding the combination to the transmission fluid, the concentration of alkoxylated alcohol reacted previously with the dispersant may range from 0.001 wt% to 50 wt%. In another embodiment, the overall concentration of the dispersant reacted with alkoxylated alcohol in the transmission fluid may range from 0.01 wt% to 20 wt%, to 15 wt%, or to 10 wt%.

Base or lubricating oils contemplated in preparing the power transmission fluids of the present invention may be derived from natural lubricating oils, synthetic lubricating oils, and mixtures thereof. Other suitable base oils may include gas to liquid base oils, and/or any base oil classified as Group I, II, III, IV, or V. In general, the base oil used in the present invention may have a kinematic viscosity at 100 °C ranging from 1.0 to 100.0 cSt, and as a further example, from 1.0 to 15.0 cSt, and as an even further example from 1.5 to 10 cSt.. Natural lubricating oils include animal oils, vegetable oils, petroleum oils, mineral oils, and oils derived from coal and shale. Mineral oils include all common mineral oil basestocks, such as naphthenic or paraffinic oils, and may have kinematic viscosities at 100 °C ranging from 0.5 to 20.0 cSt, and as a further example, from 1.5 to 15 cSt. Synthetic oils include hydrocarbon oils and halo-substituted hydrocarbon oils, such as oligomerized, polymerized, and interpolymerized olefins and alkylated diphenyl ethers, alkylated diphenyl sulfides, as well as their derivatives, analogs and homologs. Synthetic oils also include alkylene oxide polymers, interpolymers, copolymers, and derivatives thereof where the terminal hydroxyl groups have been modified by esterification, etherification, etc. Another class of synthetic lubricating oils includes the esters of dicarboxylic acids with a variety of alcohols. Silicon-based oils may also be utilized, as may liquid esters of phosphorus-containing acids, polymeric tetrahydrofurans, poly-alpha olefins, and the like. Lubricating oils may be also be derived from unrefined sources, refined oils, rerefined oils, and mixtures thereof.

In addition to the alkoxylated alcohol component, which may be optionally heated and added with an ashless dispersant, the power transmission fluid formulations of the present invention may include other optional components. These components may include other friction modifiers, dispersants, detergents, seal swell agents, antiwear agents, extreme pressure agents, antioxidants, foam inhibitors, lubricity agents, rust inhibitors, corrosion inhibitors, demulsifiers, viscosity improvers, dyes and the like. The embodiments of the present invention have been found to be effective when used in conjunction with various additives, including, for example, with and without boronated agents.

Nitrogen-containing ashless dispersants are well known as lubricating oil additives. Suitable ashless dispersants that may be used in the present invention include hydrocarbyl succinimides, hydrocarbyl succinamides, mixed ester/amides of hydrocarbyl-substituted succinic acid, and hydroxyesters of hydrocarbyl-substituted succinic acid. Also suitable in the present invention may be condensation products of polyamines and hydrocarbyl-substituted phenyl acids. Mixtures of any of these dispersants may also be used.

A method of measuring friction performance of a power transmission fluid using an LFW-1 block on ring test apparatus is described below. The method comprises applying fluids between the block and ring of the LFW-1 test apparatus. The ring is rotated relative to the block in cycles of acceleration for 40 sec from 0 to 0.5 m/sec and then deceleration from 0.5 to 0 m/sec at 121°C. The friction between the block and ring during the cycle are measured to provide 50 or more measurements, or as a further example 100 or more measurements, or as an even further example, 2800 or more measurements. A cycle may be repeated any number of times, for example, 1 to 50 times. The method may be used to measure the friction performance of a new power transmission fluid or an aged power transmission fluid to provide friction durability. To age a power transmission fluid, the fluid maybe subject to an oxidation bath for 100 hours at 170°C. The resulting friction performance measurements or friction durability may then be compared. Two or more different power transmission fluids may be so tested and then the friction performance measurements or friction durability compared. A power transmission fluid may be selected for a particular power transmitting application, such as a transmission or torque converter disclosed herein, based on the comparison of the resulting measurements. As an example, the friction performance or friction durability of a power transmission fluid comprising an alkoxylated alcohol may be compared to a power transmission fluid free of an alkoxylated alcohol. As an even further example, the friction performance or friction durability of a power transmission fluid comprising an alkoxylated alcohol may be compared to a power transmission fluid comprising a different alkoxylated alcohol.

### EXAMPLES

Transmission fluid formulations were tested and evaluated for effectiveness in modifying friction in accordance with embodiments of the present disclosure.

### EXAMPLE 1

This example demonstrates the utility of an alkoxylated alcohol additive in modifying friction initially and over time, as disclosed herein. Transmission fluid Formulation (1) was prepared as a control and contained no ELA. Formulation (1) contained an ashless dispersant at 4 wt% that contained both boron and phosphorous. Formulation (2) was prepared with 0.24 wt% ELA added directly to the transmission fluid at room temperature, and also included the ashless dispersant of Formulation (1) at 4 wt%. Formulation (3) was prepared with 6% ELA heated for 4 hours at 120°C with the ashless dispersant. The combination was then added to the other supplemental additives at an overall concentration of 4 wt% in the finished fluid.

The data shown in Table 1 were acquired using LFW-1 block on ring test apparatus using the test procedures disclosed herein. In particular, the fluids tested were applied between the block and ring of the LFW-1 test apparatus. The ring was rotated relative to the block and measurements were taken in cycles of acceleration for about 40 sec and then deceleration from about 0 to about 0.5 m/sec and back to about 0 at about 121°C. About 2800 measurements were taken per cycle. To obtain friction measurements for an aged formulation, each transmission fluid sample was "aged" for 100 hours at 170°C using an oxidation bath and subjected to the same testing conditions.

**Table 1: Effectiveness of Ethoxylated Lauryl Alcohol in Modifying Friction**

| | Static/Dynamic Initial | Static/Dynamic Aged |
|---|---|---|
| **Formulation (1)** | 0.952 | 1.057 |
| **Formulation (2)** | 0.923 | 1.031 |
| **Formulation (3)** | 0.924 | 1.024 |

In evaluating the data shown in Table 1, better friction durability is indicated by the ratio of static to dynamic friction being a number less than 1, such as 0.92. Thus, both of the formulations containing ELA surpass the control in friction durability, as the measurements for the coefficient of friction durability decrease when ELA is added to the fluid directly (Formulation (2)), and when pre-reacted with the ashless dispersant (Formulation (3)) both initially and after aging (e.g., by heating).

The data acquired during the testing of the formulations in this example are shown diagrammatically in the drawings in **FIG. 1(A)** (Initial Friction Measurements) and **FIG. 1(B)** (Aged Measurements) for the three sample formulations described above. Again, lower measurements are indicative of better friction durability; therefore, the curves achieving lower values and less change from **FIG. 1(A)** on the y-axis were indicative of better results.

Regression analysis of happenstance data from the initial LFW-1 frictional data of power transmission fluids indicated that ELA added to the fluid and ELA pre-mixed with dispersant both lower static/dynamic friction ratios with a greater than 99% probability of significance. Analysis of the frictional data obtained from testing aged fluids in the LFW-1 demonstrated that ELA added to the fluid and ELA pre-mixed with dispersant both lower static/dynamic friction ratios with a greater than 99.9% probability of significance.

### EXAMPLE 2

In another example, the LFW-1 test was run using a variety of linear-chain and branched-chain alkoxylated alcohols. The results using Samples #3-7 were compared to Sample #2, a formulation using ELA and to a formulation having no ethoxylated alcohol (Sample #1). In Sample #3, an ethoxylated C10-C12 linear alcohol with an average of 3 ethoxylations per molecule, was used. In Sample #4, an ethoxylated C10-C12 linear alcohol with an average of 5 ethoxylations per molecule, was used. In Sample #5, an ethoxylated C12-C14 linear alcohol with an average of 3 ethoxylations per molecule, was used. In Sample #6, an ethoxylated C8-C10 linear alcohol with an average of 2 ethoxylations per molecule, was used. In Sample #7, an ethoxylated C8-C10 linear alcohol with an average of 4.5 ethoxylations per molecule, was used. The formulations all contained about 4 wt% dispersant. Each formulation was tested both initially and after aging for 100 hours at 170°C. Results for the ratio of static to dynamic friction for new and aged fluid are shown, where a more desirable result is a number less than about 1. These results are also shown diagrammatically in **FIG. 2**, where the highest curve reflects results obtained from the control (no alkoxylated alcohol) sample, with the remaining curves performing similarly to ELA in friction testing.

Samples 2-7 exhibited better measures of the ratio of static to dynamic friction in comparison with the control (Sample #1). In addition, the varying alkoxylated alcohols tested in this example performed similarly to ELA.

Various branched alkoxylated alcohol samples were also tested and compared to the control sample containing no alkoxylated alcohol. Three formulations were tested which include a mixture of 50% linear and 50% branched alkoxylated alcohols. The results from testing these samples are shown in Table 2, and the results from sample #10 are shown schematically in **FIG. 3****.** In **FIG**. **3****,** curve **(a)** represents friction performance of the fluid when new and **(b)** represents friction performance of the fluid after aging. Data from an LFW-1 test were obtained using three samples: Sample #8 was a formulation comprising 3 moles of ethylene oxide per mole of alcohol, Sample #9 was a formulation comprising 5 moles of ethylene oxide per mole of alcohol, and comparative Sample #10 was a formulation comprising 7 moles of ethylene oxide per mole of alcohol. The branched alkoxylated alcohol samples achieved comparable results for friction performance to those from the ELA and linear alkoxylated alcohols tested in previous examples.

**Table 2: Comparison of Alkoxylated Alcohol Formulations**

| Sample | #1 | #2 | #3 | #4 | #5 | #6 | #7 | #8 | #9 | #10 |
|---|---|---|---|---|---|---|---|---|---|---|
| Static/Dynamic Friction (Initial) | 1.13 | 1.077 | 1.069 | 1.043 | 1.079 | 1.081 | 1.054 | 1.080 | 1.063 | 1.034 |
| Static/Dynamic Friction (Aged) | 1.113 | 1.031 | 0.997 | 0.999 | 1.036 | 1.073 | 1.027 | 1.035 | 1.004 | 0.988 |

### EXAMPLE 3

In another example, the LFW-1 test was run using samples containing varying amounts of ELA. The samples contained the same components other the varying amount of ELA. All samples included dispersant in the same amount. Sample #1 was a control and contained no ELA. Sample #2 contained 0.24 wt% ELA, Sample #3 contained 0.48 wt% ELA, Sample #4 contained 1.5 wt% ELA, and Sample #5 contained 3.0 wt% ELA. The formulations were tested initially and after aging for 100 hours at 170°C. Results for the ratio of static to dynamic friction for new and aged fluid are shown in Table 3, where a more desirable result is a number less than 1. The results indicate improving static/dynamic friction ratios in the aged samples as the ELA is present and is increased.

**Table 3: Comparison of Various Amounts of ELA**

| Sample | #1 | #2 | #3 | #4 | #5 |
|---|---|---|---|---|---|
| Static/Dynamic Friction (Initial) | 0.952 | 0.965 | 0.97 | 0.938 | 0.946 |
| Static/Dynamic Friction (Aged) | 1.057 | 1.034 | 1.01 | 0.958 | 0.914 |

### EXAMPLE 4

A regression analysis of happenstance data was also performed on samples containing ELA added as a component and ELA pre-reacted with a dispersant using an LVFA Durability test (JASO M349). The data indicated with a greater than 95% probability of significance that the use of ELA is effective in extending durability life of a power transmission fluid including the same. The same analysis showed with a greater than 99% probability that ELA pre-mixed with dispersant also has a positive effect on durability life.

As used throughout the specification and claims, "a" and/or "an" may refer to one or more than one. At the very least, and not as an attempt to limit the application of the doctrine of equivalents to the scope of the claims, each numerical parameter should at least be construed in light of the number of reported significant digits and by applying ordinary rounding techniques. Notwithstanding that the numerical ranges and parameters setting forth the broad scope of the invention are approximations, the numerical values set forth in the specific examples are reported as precisely as possible. Any numerical value, however, inherently contains certain errors necessarily resulting from the standard deviation found in their respective testing measurements.

## Claims

1. A power transmission fluid, including:
(a) a major amount of a base oil; and
(b) a minor amount of an additive composition including:
at least one alkoxylated alcohol of the formula R-[O-(CH₂)_{X}]_{Y}-OH, wherein R is an aliphatic hydrocarbon group having from 8 to 18 carbon atoms, X is 2 to 4, and Y is 1 to 6; and
a dispersant selected from a hydrocarbyl succinimide, a hydrocarbyl succinamide, a mixture of an ester and an amide of a hydrocarbyl-substituted succinic acid, and a hydroxyester of a hydrocarbyl-substituted succinic acid; wherein the power transmission fluid includes 0.01 to 20 wt% of the alkoxylated alcohol and 0.01 to 15 wt% of the dispersant, based on the total weight of the fluid.

2. The fluid of claim 1, wherein the aliphatic hydrocarbon is a saturated or unsaturated linear, branched, or cyclic hydrocarbon.

3. The fluid of claim 1, wherein the alkoxylated alcohol has at least eight carbon atoms.

4. The fluid of any one of claims 1-3, wherein the amount of alkoxylated alcohol in the fluid is 0.01 wt% to 10 wt%, based on the total weight of the fluid.

5. The fluid of any one of claims 1-3, wherein the amount of alkoxylated alcohol in the fluid is 0.05 wt% to 6 wt%, based on the total weight of the fluid.

6. The fluid of any one of claims 1-3, wherein the amount of alkoxylated alcohol in the fluid is 0.1 wt% to 3 wt%, based on the total weight of the fluid.

7. The fluid of any one of claims 1-6, wherein the base oil includes one or more of a natural lubricating oil, a synthetic lubricating oil, and mixtures thereof.

8. The fluid of any one of claims 1-7, wherein the fluid is a belt, chain, or disk-type continuously variable transmission fluid.

9. The fluid of claim 1, wherein the concentration of the dispersant in the fluid is 0.01 wt% to 10 wt%, based on the total weight of the fluid.

10. The fluid of any one of claims 1-9, wherein the fluid has improved friction durability relative to a fluid having the same composition absent said at least one alkoxylated alcohol, and wherein said friction durability is measured by applying the fluid between a block and ring of an LFW-1 test apparatus, and (1) rotating the ring relative to the block in a cycle of acceleration for 40 seconds from 0 to 0.5 m/sec and then deceleration from 0.5 to 0 m/sec at 121°C, (2) measuring friction between the block and ring during the cycle and (3) repeating steps (1)-(3) for 2800 or more measurements.

11. A method of operating a power transmission to increase the duration of friction-modifying capabilities of a power transmission fluid, said method including the steps of adding to the power transmission a power transmission fluid as claimed in any one of claims 1-10, and operating the power transmission.

12. A method of operating a power transmission as claimed in claim 11, wherein the power transmission is a continuously variable transmission.

13. Use of an additive composition including 0.01 to 20 wt % of at least one alkoxylated alcohol of the formula R-[O-(CH₂)_{X}]_{Y}-OH, wherein R is an aliphatic hydrocarbon group having from 8 to 18 carbon atoms, X is 2 to 4, and Y is 1 to 6 to increase a duration of friction-modifying capabilities of a power transmission fluid including 0.01 to 15 wt.% of a dispersant, said weight percentages being based on the total weight of the fluid.

14. Use as claimed in claim 13, wherein the dispersant includes one or more of a hydrocarbyl succinimide, a hydrocarbyl succinamide, a mixture of an ester and an amide of a hydrocarbyl-substituted succinic acid, and a hydroxyester of a hydrocarbyl-substituted succinic acid.

## Patentansprüche

1. Ein Leistungsgetriebefluid umfassend:
(a) eine Hauptmenge eines Grundöls; und
(b) eine Nebenmenge einer Additivzusammensetzung umfassend:
mindestens einen alkoxylierten Alkohol der Formel R-[O-(CH₂)_{X}]_{Y}-OH, wobei R eine Gruppe aliphatischer Kohlenwasserstoffe mit 8 bis 18 Kohlenstoffatomen, X 2 bis 4 und Y 1 bis 6 ist; und
ein Dispergiermittel ausgewählt aus einem Hydrocarbylsuccinimid, einem Hydrocarbylsuccinamid, einer Mischung eines Esters und eines Amids einer Hydrocarbyl-substituierten Bernsteinsäure und einem Hydroxyester einer Hydrocarbyl-substituierten Bernsteinsäure;
wobei das Leistungsgetriebefluid 0,01 bis 20 Gew.-% des alkoxylierten Alkohols und 0,01 bis 15 Gew.-% des Dispergiermittels bezogen auf das Gesamtgewicht des Fluids umfasst.

2. Das Fluid gemäß Anspruch 1, wobei der aliphatische Kohlenwasserstoff ein gesättigter oder ungesättigter geradkettiger, verzweigter oder cyclischer Kohlenwasserstoff ist.

3. Das Fluid gemäß Anspruch 1, wobei der alkoxylierte Alkohol mindestens acht Kohlenstoffatome aufweist.

4. Das Fluid gemäß irgendeinem der Ansprüche 1-3, wobei sich die Menge des alkoxylierten Alkohols im Fluid auf 0,01 Gew.-% bis 10 Gew.-% bezogen auf das Gesamtgewicht des Fluids beläuft.

5. Das Fluid gemäß irgendeinem der Ansprüche 1-3, wobei sich die Menge des alkoxylierten Alkohols im Fluid auf 0,05 Gew.-% bis 6 Gew.-% bezogen auf das Gesamtgewicht des Fluids beläuft.

6. Das Fluid gemäß irgendeinem der Ansprüche 1-3, wobei sich die Menge des alkoxylierten Alkohols im Fluid auf 0,1 Gew.-% bis 3 Gew.-% bezogen auf das Gesamtgewicht des Fluids beläuft.

7. Das Fluid gemäß irgendeinem der Ansprüche 1-6, wobei das Grundöl eines oder mehr eines natürlichen Schmieröls, eines synthetischen Schmieröls und Mischungen daraus umfasst.

8. Das Fluid gemäß irgendeinem der Ansprüche 1-7, wobei das Fluid ein Fluid für stufenlose Riemen-, Ketten- oder Scheibengetriebe ist.

9. Das Fluid gemäß Anspruch 1, wobei die Konzentration des Dispergiermittels im Fluid 0,01 Gew.-% bis 10 Gew.-% bezogen auf das Gesamtgewicht des Fluids beträgt.

10. Das Fluid gemäß irgendeinem der Ansprüche 1-9, wobei das Fluid eine verbesserte Reibungsbeständigkeit hat in Relation zu einem Fluid, das die gleiche Zusammensetzung ohne besagten mindestens einen alkoxylierten Alkohol aufweist, und wobei die besagte Reibungsbeständigkeit gemessen wird durch Aufbringen des Fluids zwischen einem Block und einem Ring einer LFW-1-Prüfvorrichtung und durch (1) Drehen des Rings in Relation zum Block in einem 40 Sekunden dauernden Zyklus aus Beschleunigung von 0 auf 0,5 m/s und dann Entschleunigung von 0,5 auf 0 m/s bei 121 °C, (2) Messen der Reibung zwischen dem Block und dem Ring während des Zyklus und (3) Wiederholen der Schritte (1)-(3) für mindestens 2800 Messungen.

11. Ein Verfahren zum Betrieb eines Leistungsgetriebes zur Verlängerung der Dauer reibungsmodifizierender Fähigkeiten eines Leistungsgetriebefluids, wobei besagtes Verfahren die Schritte des Hinzufügens eines Leistungsgetriebefluids gemäß irgendeinem der Ansprüche 1-10 zum Leistungsgetriebe umfasst sowie den Betrieb des Leistungsgetriebes.

12. Ein Verfahren zum Betrieb eines Leistungsgetriebes gemäß Anspruch 11, wobei das Leistungsgetriebe ein stufenloses Getriebe ist.

13. Anwendung einer Additivzusammensetzung umfassend 0,01 bis 20 Gew.-% von mindestens einem alkoxylierten Alkohol der Formel R-[O-(CH₂)_{X}]_{Y}-OH, wobei R eine Gruppe aliphatischer Kohlenwasserstoffe mit 8 bis 18 Kohlenstoffatomen, X 2 bis 4 und Y 1 bis 6 ist, zur Verlängerung einer Dauer reibungsmodifizierender Fähigkeiten eines Leistungsgetriebefluids umfassend 0,01 bis 15 Gew.-% eines Dispergiermittels, wobei die besagten Gewichtsprozentsätze auf das Gesamtgewicht des Fluids bezogen sind.

14. Anwendung gemäß Anspruch 13, wobei das Dispergiermittel eines oder mehr von einem Hydrocarbylsuccinimid, einem Hydrocarbylsuccinamid, einer Mischung eines Esters und eines Amids einer Hydrocarbyl-substituierten Bernsteinsäure und einem Hydroxyester einer Hydrocarbyl-substituierten Bernsteinsäure umfasst.

## Revendications

1. Un fluide de transmission de puissance, comprenant :
(a) une quantité majeure d'une d'huile de base ; et
(b) une quantité mineure d'une composition d'additifs comprenant :
au moins un alcool alcoxylé de formule R-[O-(CH₂)ₓ]_{y}-OH, **caractérisé en ce que** R est un radical hydrocarboné aliphatique comprenant 8 à 18 atomes de carbone, x est compris entre 2 et 4 et y est compris entre 1 et 6 ; et
un agent dispersant pouvant être un succinimide d'hydrocarbyle, un succinamide d'hydrocarbyle, un mélange d'un ester et d'un amide d'acide succinique substitué par un groupe hydrocarbyle, un hydroxyester d'acide succinique substitué par un groupe hydrocarbyle ;
**caractérisé en ce que** le fluide de transmission de pussance contient 0,01 à 20 % en poids d'alcool alcoxylé et 0,01 à 15 % en poids d'agent dispersant, sur la base du poids total du fluide.

2. Le fluide selon la revendication 1, **caractérisé en ce que** le radical hydrocarboné aliphatique peut être un hydrocarbure linéaire, ramifié ou cyclique, saturé ou insaturé.

3. Le fluide selon la revendication 1, **caractérisé en ce que** l'alcool alcoxylé comprend au moins huit atomes de carbone.

4. Le fluide selon l'une quelconque des revendications 1 à 3, **caractérisé en ce que** la quantité d'alcool alcoxylé dans le fluide est comprise entre 0,01 et 10 % en poids, sur la base du poids total du fluide.

5. Le fluide selon l'une quelconque des revendications 1 à 3, **caractérisé en ce que** la quantité d'alcool alcoxylé dans le fluide est comprise entre 0,05 et 6 % en poids, sur la base du poids total du fluide.

6. Le fluide selon l'une quelconque des revendications 1 à 3, **caractérisé en ce que** la quantité d'alcool alcoxylé dans le fluide est comprise entre 0,1 et 3 % en poids, sur la base du poids total du fluide.

7. Le fluide selon l'une quelconque des revendications 1 à 6, **caractérisé en ce que** l'huile de base contient au moins une huile lubrifiante naturelle, une huile lubrifiante synthétique, ou un mélange de celles-ci.

8. Le fluide selon l'une quelconque des revendications 1 à 7, **caractérisé en ce que** le fluide est un fluide pour transmission à variation continue de type à courroie, chaîne ou disque.

9. Le fluide selon la revendication 1, **caractérisé en ce que** la concentration d'agent dispersant dans le fluide est comprise entre 0,01 et 10 % en poids, sur la base du poids total du fluide.

10. Le fluide selon l'une quelconque des revendications 1 à 9, **caractérisé en ce que** le fluide présente une meilleure résistance aux frottements qu'un fluide de même composition hormis au moins un alcool alcoxylé, et **caractérisé en ce que** ladite résistance aux frottements est mesurée en appliquant le fluide entre le bloc et l'anneau d'un appareil d'essai LFW-1, et (1) en faisant tourner l'anneau par rapport au bloc selon un cycle comprenant une accélération de 0 à 0,5 m/s pendant 40 secondes puis une décélération de 0,5 à 0 m/s à 121 °C ; (2) en mesurant les frottements entre le bloc et l'anneau pendant le cycle ; et (3) en répétant les étapes (1) et (3) pendant au moins 2800 mesures.

11. Une méthode d'exploitation d'un transmission de puissance visant à augmenter la durée des capacités de modification des frottements d'un fluide de transmission de puissance, les étapes de ladite méthode comprenant l'ajout d'un fluide de transmission de puissance dans le transmission de puissance selon l'une quelconque des revendications 1 à 10, et l'exploitation du transmission de puissance.

12. Une méthode d'exploitation d'un transmission de puissance selon la revendication 11, **caractérisée en ce que** le transmission de puissance est une transmission à variation continue.

13. L'utilisation d'une composition d'additifs contenant 0,01 à 20 % en poids d'au moins un alcool alcoxylé de formule R-[O-(CH₂)ₓ]_{y}-OH, **caractérisé en ce que** R est un radical hydrocarboné aliphatique comprenant 8 à 18 atomes de carbone, x est compris entre 2 et 4 et y est compris entre 1 et 6, afin d'augmenter la durée des capacités de modification des frottements d'un fluide de transmission de puissance contenant 0,01 à 15 % en poids d'un agent dispersant, lesdits pourcentages massiques étant basés sur le poids total du fluide.

14. L'utilisation selon la revendication 13, **caractérisée en ce que** l'agent dispersant comprend au moins un succinimide d'hydrocarbyle, un succinamide d'hydrocarbyle, un mélange d'un ester et d'un amide d'acide succinique substitué par un groupe hydrocarbyle, ou un hydroxyester d'acide succinique substitué par un groupe hydrocarbyle.
